

## UNITED STATES PATENT OFFICE.

ELIAS ANTHON CAPPELEN SMITH, OF NEW YORK, N. Y.

## METALLURGY OF TIN.

No Drawing.

Application filed January 16, 1923. Serial No. 613,052.

*To all whom it may concern:*

Be it known that I, ELIAS ANTHON CAPPELEN SMITH, a citizen of the United States, residing at New York city, in the county of 5 New York, State of New York, have invented certain new and useful Improvements in Metallurgy of Tin; and I do hereby declare the following to be a full, clear, and exact description of the invention, such 10 as will enable others skilled in the art to which it appertains to make and use the same.

This invention relates to the recovery of tin from ores and other tin-containing materials. More particularly the invention relates to a process of recovering tin from materials with which it is mixed and from which it cannot be separated readily by ordinary metallurgical treatment. It is 20 especially applicable to the treatment of low grade tin ores but may be employed also in treating higher grade ores and various materials containing tin or tin compounds.

The smelting of tin ores in ordinary shaft or reverberatory furnaces is not accomplished with the ease which characterizes the separation of copper or lead from ores containing these elements. The higher oxide of tin ( $\text{SnO}_2$ ) is not dissociated 25 readily into the lower oxide ( $\text{SnO}$ ) and oxygen by heat alone at the temperatures usually prevailing in the furnace. Consequently the distribution of oxygen is not easily accomplished, and special precautions are 30 necessary to ensure effective smelting. Thus in reverberatory smelting only the surface of the charge receives enough oxygen for proper combustion of the carbonaceous reducing agent, and it is necessary 35 to rabble the charge constantly so that fresh material is brought to the surface in contact with the oxygen. There is a tendency, moreover, for the charge to fuse at the temperature at which carbon monoxide is produced (about  $1100^\circ \text{C}$ ), and fusion renders 40 the charge less pervious and reduces the efficiency of the operation. This difficulty is met in shaft as well as in reverberatory furnaces. In either practice the first slag contains generally 20 to 40 per cent of tin, owing to inability of the oxygen to permeate 45 the charge and to the tendency of the tin to combine with the gangue and the fluxing agents employed.

50 It is the object of the present invention to avoid the difficulties which are met in smelting tin ores as heretofore practiced and to provide a process whereby tin may be recovered in an efficient and relatively inexpensive manner from tin-bearing materials, particularly from low grade or refractory ores. The application of the invention permits recovery of upward to 93 to 95 per cent of the tin in ores containing 5 to 6 per cent of tin.

In general the process depends upon the preliminary treatment of the ore or other material at temperatures much lower than those employed in ordinary smelting to bring the tin into a condition in which it is 60 readily soluble in solvents from which it may be separated by electrolysis. This preliminary treatment may be omitted if the tin is already in soluble form. Such treatment may include roasting, although this is 65 not necessary with many tin-bearing materials. The ore or tin-bearing material, either with or without previous roasting, is crushed to a suitable degree of fineness (e. g., 70 20 mesh) and treated to bring the tin into 75 soluble condition, for example, by reduction with a gaseous reducing agent or by sulphidizing. Reduction may be accomplished by heating the material to about 80  $800^\circ \text{C}$ . to  $850^\circ \text{C}$ . with any suitable gas such as hydrogen, water gas, or gases produced 85 from coal, oil or other fuel. Sulphidizing may be carried out by conducting sulphur vapor from a convenient source into contact with the heated ore. These operations are 90 continued for appropriate periods to ensure the accomplishment of the desired result.

When the tin content of the ore or material has been brought to the state in which it is 95 soluble (if it is not naturally in that state) the material is leached with a solvent. Such a solvent may be a dilute sulphuric acid solution (e. g., 150 grams  $\text{H}_2\text{SO}_4$  per liter) containing 10 to 20 grams per liter of tin as stannic sulphate and 10 to 50 grams per liter 100 of iron, chiefly as ferric sulphate. During the leaching the stannic tin and ferric iron are largely reduced to stannous tin and ferrous iron, and metallic tin is dissolved. The sulphuric acid dissolves a portion of the tin.

The tin-containing solution may be electrolyzed, using a lead anode and an ordinary current density of 10 to 20 amperes per square foot. Sheet tin forms a suitable cathode. As the tin is deposited on the cathode the solvent is regenerated by the oxidation 105 of the tin and iron compounds, and the

solution may be returned for the treatment of further quantities of tin-bearing materials. The solvent may be used repeatedly in this way until it accumulates a proportion 5 of iron which renders it ineffective. All of the tin is then separated and the iron-containing acid must be replaced with fresh acid.

This difficulty is avoided by the use of a 10 solvent containing a soluble polysulphide, for example, an alkali metal polysulphide, which selectively dissolves tin without taking up iron from the tin-containing material. A suitable solvent contains 100 grams 15 of sodium sulphide and 30 grams of sulphur per liter. The solvent is regenerated by electrolyzing to deposit the tin. Lead or iron anodes may be employed with a current density of about 30 amperes per square foot 20 at a temperature of 20° C. to 60° C. The solvent may contain 30 to 40 grams of tin per liter before electrolysis, and 10 to 20 grams of tin per liter when it is returned for reuse in leaching the tin-bearing material. 25

The soluble polysulphide solvent is particularly useful in connection with the sulphidizing of the tin. The tin, instead of being reduced to the metallic state, is converted 30 into the sulphide which is soluble readily in the sodium polysulphide solution. Under certain conditions where sulphur is cheaply available and fuel is expensive, the process described is particularly efficient and 35 desirable.

Soluble hydroxides, for example, alkali metal hydroxides, may also be used as a solvent for the treatment of material in which the tin has been reduced to the metallic condition. The tin is less readily separated 40 from the hydroxide solution, and a mixture of sodium hydroxide and sodium polysulphide is more desirable, the hydroxide serving to neutralize any tendency of 45 the polysulphide to become acidic after repeated use. Soluble hydroxides, sulphides, polysulphides or mixtures of these are suitable solvents.

The most effective gaseous reducing agent 50 for the practice of the invention is hydrogen which may be obtained from any suitable source, by electrolysis of water, for example. Many gases containing hydrogen, carbon monoxide or hydrocarbons or mixtures thereof may be used in place of hydrogen. Thus, to mention a few available gases, 55 water gas, producer gas, illuminating gas, oil gas or hydrocarbon vapors may be employed.

For the proper conduct of the reducing 60 or sulphidizing operations suitable apparatus must be provided. In reducing iron furnaces or retorts may be used at the relatively low temperatures employed. It may be desirable, however, to use retorts or furnaces

of iron lined with refractory material such as magnesite or with a corrosion-resistant material such as an alloy of iron and chromium containing not less than 30 per cent of chromium. Such alloys may contain upward to 60 per cent of chromium, and the entire furnace or retort, or any part thereof, may be constructed of this material. Alloys of iron with other elements such as titanium, uranium, vanadium and manganese may also be employed in furnaces and retorts suitable for the purpose of the invention. 70 75

Electrolytic cells of the usual types may be employed in carrying out the electrolysis. 80 These cells may be equipped with diaphragms or not, depending upon special conditions affecting the operation. The cells and other apparatus used, being of well known construction, are not a part of the 85 invention and are not described.

These and other details of the operation may vary, the specific examples being illustrative merely and are not intended as indicating the limits of the invention. Such variations are within the spirit of the invention and the scope of the accompanying claims.

I claim:—

1. The process of recovering tin from low grade tin-bearing material which comprises subjecting the material to the action of a gaseous reducing agent whereby the compounds of tin in the material are reduced, dissolving the tin in the thus-treated material by means of an appropriate solvent, and recovering tin from the resulting solution by electrodeposition.

2. The process of recovering tin from tin-bearing material, which comprises subjecting the material to the action of a gaseous reducing agent whereby the compounds of tin in the material are reduced, dissolving the tin in the thus-treated material by means of an appropriate solvent, recovering tin 103 from the resulting solution by electrodeposition, and returning the spent electrolyte 110 for the solution of further tin from similarly treated tin-bearing material.

3. The process of recovering tin from tin-bearing material, which comprises dissolving the tin in a solution containing a soluble polysulphide and electrolyzing the solution to separate the tin. 115

4. The process of recovering tin from tin-bearing material, which comprises subjecting the material to the action of a gaseous reducing agent, dissolving the tin in the thus-treated material by means of a solvent which is capable of regeneration by the electrodeposition of tin therefrom, recovering tin from the resulting solution by electrodeposition, and returning the spent electrolyte 120 for the solution of further tin from similarly treated tin-bearing material. 125 130

5. The process of recovering tin from tin-bearing material, which comprises subjecting the material to the action of a reducing gas, dissolving the tin with a solvent which 5 is capable of regeneration by electrolytic treatment to deposit tin therefrom, and electrolyzing the solution to separate the tin.

6. The process of recovering tin from tin-bearing material, which comprises subjecting the material to the action of sulphur vapors, dissolving the tin with a solvent which is capable of regeneration by electrolytic treatment to deposit tin therefrom, 15 and electrolyzing the solution to separate the tin.

7. The process of recovering tin from tin-bearing material, which comprises subjecting the material to a preliminary treatment for rendering the tin content of the 20 material more amenable to solution in an appropriate solvent capable of regeneration by the electrodeposition of tin therefrom, dissolving the tin in the thus-treated material by means of an appropriate solvent 25 of the aforesaid character, and recovering tin from the resulting solution by electrodeposition.

8. The process of recovering tin from tin-bearing material, which comprises subjecting the material to a preliminary treatment to make the tin soluble, dissolving the 30 tin in a solution containing a soluble polysulphide, and electrolyzing the solution to 35 separate the tin.

9. The process of recovering tin from tin-bearing material, which comprises subjecting the material to the action of a gaseous reducing agent whereby the compounds of tin are reduced, dissolving the tin in the 40 thus-treated material by means of an appropriate solvent solution containing a soluble polysulfide, and recovering tin from the resulting solution by electrodeposition.

10. The process of recovering tin from 45 tin-bearing material, which comprises subjecting the material to preliminary treatment for rendering the tin content thereof more amenable to solution in a solvent containing a soluble polysulfide, dissolving the 50 tin in the thus-treated material by means of a solvent solution containing a soluble polysulfide, recovering tin from the resulting solution by electrodeposition, and returning the spent electrolyte for the 55 solution of further tin from similarly treated tin-bearing material.

11. The process of recovering tin from tin-bearing material, which comprises subjecting the material at an elevated temperature to the action of a gaseous reducing agent, dissolving the tin in the thus-treated material by means of a solvent solution containing a soluble polysulfide, and recovering 60 tin from the resulting solution by electrodeposition.

In testimony whereof I affix my signature.

ELIAS ANTHON CAPPELEN SMITH.